

## UNITED STATES PATENT OFFICE

2,515,181

METHOD OF TREATING WOOL AND FABRICS  
FORMED THEREFROM TO INCREASE  
THEIR RESISTANCE TO DECOMPOSITION  
BY HEATCharles R. Barnes, Pittsburgh, Pa., assignor to  
Albany Felt Company, Albany, N. Y., a corpora-  
tion of New YorkNo Drawing. Application April 13, 1948,  
Serial No. 20,848

15 Claims. (Cl. 8—128)

1

Many fabrics formed entirely or in substantial part of wool fibers are used in the mechanical arts for purposes where they are subjected to elevated temperatures. For example, fabrics used for filtering chemicals, or as slasher cloth for applying sizing material to yarns or fabrics, are often subjected to temperatures near the boiling point of water. Fume bags are used for collecting dust from air at temperatures often as high as 250° to 300° F. Some fabrics are used for filtering oils at temperatures as high as 350° F., while others are used for applying paraffin coatings at high temperatures to milk bottle caps, paperboard containers, and the like. Blankets, such as Sanforizing blankets, which are used in shrinking other fabrics, are also subjected to comparatively high temperatures while in a moist condition. Thus, many wool fabrics are subjected both to dry heat and to heat while wet or moistened with various liquid media.

Wool fibers when subjected to temperatures of the above order decompose quite rapidly, depending upon temperature and other conditions, with the result that the life of the fabrics formed therefrom is comparatively short.

Therefore, the principal object of my invention is to provide a comparatively simple treatment whereby the resistance to heat of wool fabrics formed therefrom is substantially increased. It is to be understood that my invention is not limited in its application to fabrics formed entirely of wool, because it may be applied to fabrics formed in part of wool and other fibers, such as cotton, rayon, nylon and the like, for increasing the resistance to heat of the wool content thereof. The wool may be processed at almost any stage of its fabrication into a textile. Thus, the treatment may be applied to the scoured raw wool, to the yarn, or to the fabric after it is formed. I prefer, however, to treat the woven fabric since it is most convenient to process the wool when in this form.

I have discovered that the heat resistance of wool is improved to a greater or lesser extent by treatment in water solution with the complex thiocyanate ions of such metals as form complex metallo-thiocyanate ions in the solution. Those thiocyanates which form the more symmetrical thiocyanate complex ions are more effective than those which form complex ions of the asymmetrical type. The general type of the metallo-thiocyanate complex ions may be represented by the formula  $[M(SCN)_n]^e$ , in which M is a metal, n the number of thiocyanate groups contained by the ion, and e the quantity of negative charge upon the ion. The value of e is found by subtracting n from the valence of the metal. When the numerical value of e is an even number, a

2

more symmetrical type of thiocyanate complex ion is formed than when e is odd. For instance, zinc or cadmium thiocyanates in water solution form symmetrical complex ions which may be represented in the case of the zinc salt as follows:



Examples of the asymmetrical type of complex ions are those formed by ferric, aluminum or chromium thiocyanates which may be represented in the case of the ferric salt as follows:



Such negatively charged complex ions evidently form metallo-thiocyanate cross linkages between the polypeptide chains at positive groups in the wool, thus producing a modified wool which is more resistant to decomposition by heat.

The effectiveness of the thiocyanate complex also depends on the radius of the ion, its solubility, and its stability as well as the stability of the metallo-thiocyanate complex formed with the wool. For instance the symmetrical zinc thiocyanate complex ion apparently has the optimum diameter to produce the most effective metallo-thiocyanate-wool complex. Cadmium whose ions are larger than those of zinc is slightly less effective, and, consequently, all other metals of greater atomic diameter than zinc are much less effective.

Regarding those metals whose atomic radii are less than that of zinc and which are capable of forming stable symmetrical thiocyanate complex ions in water solution, I have found that cupric thiocyanate is quite effective in protecting wool against the action of wet heat but less effective against the action of dry heat, where, apparently, the wool-cupric thiocyanate complex decomposes at elevated temperatures. Likewise, beryllium, whose ions are much smaller than those of zinc, also forms a metallo-thiocyanate-wool complex which is quite effective against decomposition by wet heat but less effective against the action of dry heat.

Evidence, including X-ray diffraction patterns, indicates that the metal thiocyanate forms a cross-linkage at the amino groups of the wool thus leaving the disulfide linkages intact. In other words, the thiocyanate chemically combines with the wool to form therewith an organic, metallo-thiocyanate complex.

In practice, the fabric to be treated may be loaded into a dye tub containing water where it may be run over a roll and into the solution in the bottom of the tub. Heat, such as may be supplied by discharging steam into the water, is applied until the temperature is in the approximate range of 115 to 120° F. When the fabric is

thoroughly wet, the chemicals are added to the water in the same way that dyes are normally added in the dyeing of fabrics. That is to say, they are added gradually over a period of perhaps 10 to 30 minutes and at a rate which is adapted to permit the fabric to pick them up gradually and uniformly. The fabric is then run through the solution which is maintained at approximately 115° F., until the fibers of the wool have had sufficient time to become thoroughly saturated and to react with the chemical in the solution. At 115° F., satisfactory saturation may be effected in about two hours. After the treatment, the fabric is extracted, dried, and finished in the normal way.

Instead of treating the woven fabric, the wool, as pointed out above, may be treated after it is scoured, or after it has been made into yarn. This can be done in a number of ways, but the important features to be observed in all cases are that the material treated is brought into intimate contact with the treating solution, and that some relative motion between the wool and the solution take place during the treatment.

The temperature of the solution is not critical because the treatment may be carried out with the solution at room temperatures or at temperatures considerably higher than the range mentioned above. At lower temperatures a longer time is required in order to effect an equivalent degree of treatment and, at higher temperatures, less time is required but, if the temperature is too high, some deterioration of the fabric may result therefrom. The temperature range of 115 to 120° F., is preferred because it allows practical speed without appreciable adverse effect on the fabric.

The quantity of chemical necessary to improve the heat resistance of the wool varies over a considerable range depending on the temperatures at which the treatment is conducted, the duration therefrom, etc. A solution containing, by weight, as little as 0.07% has some beneficial effect, and as much as 20% or more may be used. However, from 1% to 3% is sufficient to treat the wool effectively when applied for two hours at 115° F., and is therefore preferred in the practical application of my process.

The tests set forth in Tables I and II below indicate that the foregoing treatment makes the fabric substantially more resistant to both wet and dry heat than an untreated fabric.

Table I

| Trial No. | Treatment                                                                 | Tensile Strength, Pounds | Per Cent improvement |
|-----------|---------------------------------------------------------------------------|--------------------------|----------------------|
| 42        | Untreated                                                                 | 70.2                     |                      |
| 44        | 2% (ZnCl <sub>2</sub> +NH <sub>4</sub> SCN)                               | 81.9                     | 16.7                 |
| 45        | 2% (ZnAc <sub>2</sub> +NH <sub>4</sub> SCN)                               | 83.1                     | 18.4                 |
| 46        | 2% (ZnSiF <sub>6</sub> +NH <sub>4</sub> SCN)                              | 79.3                     | 13.0                 |
| 47        | 2% (Zn(NO <sub>3</sub> ) <sub>2</sub> +NH <sub>4</sub> SCN)               | 82.4                     | 17.7                 |
| 48        | 2% (ZnI <sub>2</sub> +NH <sub>4</sub> SCN)                                | 81.7                     | 16.4                 |
| 49        | 2% (ZnSO <sub>4</sub> +NaSCN)                                             | 84.8                     | 20.8                 |
| 50        | 2% (ZnSO <sub>4</sub> +NH <sub>4</sub> SCN)                               | 82.7                     | 18.0                 |
| 51        | 2% (ZnCl <sub>2</sub> +NaSCN)                                             | 85.8                     | 22.0                 |
| 71        | 2% (Al <sub>2</sub> (SO <sub>4</sub> ) <sub>3</sub> +NH <sub>4</sub> SCN) | 77.5                     | 10.4                 |
| 201       | 0.1% (CdCl <sub>2</sub> +NH <sub>4</sub> SCN)                             | 81.0                     | 15.2                 |
| 202       | 0.1% (ZnCl <sub>2</sub> +NH <sub>4</sub> SCN)                             | 80.1                     | 14.0                 |
| 203       | 0.07% (CdCl <sub>2</sub> +NH <sub>4</sub> SCN)                            | 75.5                     | 7.4                  |
| 204       | 0.07% (ZnCl <sub>2</sub> +NH <sub>4</sub> SCN)                            | 78                       | 11.4                 |
| 205       | 20% (CdCl <sub>2</sub> +NH <sub>4</sub> SCN)                              | 85.3                     | 21.3                 |
| 206       | 20% (ZnCl <sub>2</sub> +NH <sub>4</sub> SCN)                              | 88.6                     | 26.1                 |

## NOTES:

- All of the above samples were submerged in distilled water for 6 hours at 209° F. before they were tested.
- The percent of the chemicals refers to that of the metal thiocyanate calculated stoichiometrically from the salts indicated.

Table II

| Trial No. | Treatment                                                  | Tensile Strength, Pounds | Per Cent improvement |
|-----------|------------------------------------------------------------|--------------------------|----------------------|
| 5         | 113 Untreated                                              | 65.2                     |                      |
|           | 0.1% (ZnAc <sub>2</sub> +NH <sub>4</sub> SCN)              | 67.8                     | 4.0                  |
|           | 0.5% (ZnAc <sub>2</sub> +NH <sub>4</sub> SCN)              | 78.2                     | 19.9                 |
|           | 1.0% (ZnAc <sub>2</sub> +NH <sub>4</sub> SCN)              | 87.0                     | 33.4                 |
|           | 2.0% (ZnAc <sub>2</sub> +NH <sub>4</sub> SCN)              | 94.6                     | 45.1                 |
|           | 5.0% (ZnAc <sub>2</sub> +NH <sub>4</sub> SCN)              | 100.2                    | 53.7                 |
|           | 10.0% (ZnAc <sub>2</sub> +NH <sub>4</sub> SCN)             | 98.5                     | 51.1                 |
|           | 2.0% (Cr <sub>2</sub> O <sub>3</sub> +NH <sub>4</sub> SCN) | 68.5                     | 5.1                  |
|           | 2.0% (CdCl <sub>2</sub> +NH <sub>4</sub> SCN)              | 85.6                     | 31.3                 |
|           | 2.0% (NiCrO <sub>4</sub> +NH <sub>4</sub> SCN)             | 66.9                     | 2.6                  |
|           | 2.0% (Fe(SCN) <sub>3</sub> )                               | 81.2                     | 24.5                 |
|           | 0.1% (CdCl <sub>2</sub> +NH <sub>4</sub> SCN)              | 79.3                     | 21.8                 |
|           | 0.1% (ZnCl <sub>2</sub> +NH <sub>4</sub> SCN)              | 78.8                     | 21.0                 |
|           | 0.07% (CdCl <sub>2</sub> +NH <sub>4</sub> SCN)             | 66.0                     | 1.0                  |
|           | 0.07% (ZnCl <sub>2</sub> +NH <sub>4</sub> SCN)             | 65.3                     | 0.0                  |
|           | 20% (CdCl <sub>2</sub> +NH <sub>4</sub> SCN)               | 88.5                     | 36                   |
|           | 20% (ZnCl <sub>2</sub> +NH <sub>4</sub> SCN)               | 108.8                    | 67                   |

## NOTES:

- All of the above tests were subjected to dry heat at 284° F. for 24 hours before they were tested.
- The percent of the chemicals refers to that of the metal thiocyanate calculated from the salts indicated stoichiometrically.

Other tests, in which specimens of treated and untreated wool were subjected to dry heat at 284° F., for 24 hours, the gases given off by the wool collected by continually sweeping them from the heated wool, passing them through wash bottles, and thereafter analyzing them, indicate that very much less sulfur and nitrogen are lost by the treated wool than by the untreated wool.

The following is a typical example of the losses of sulfur and nitrogen sustained by the treated and untreated samples which were subjected to the dry heat mentioned above.

| Treatment               | Per Cent Sulfur Lost | Per Cent Ammonia Lost |
|-------------------------|----------------------|-----------------------|
| None                    | 0.0095               | 0.0569                |
| 2% Zn(SCN) <sub>2</sub> | 0.0933               | 0.0140                |

X-ray diffraction patterns indicate that there is no change in the side chain spacing between the treated and untreated wool in either the slack condition or when stretched 45%. This would indicate that the treating chemicals have been added to the amino groups rather than breaking the disulfide bonds.

As pointed out above, the preferred metal salts are the zinc and cadmium thiocyanates. It is not necessary that these salts be added as such to the water but only that the thiocyanate ions and the metal ions be present in the same solution. This, ammonium thiocyanate with zinc chloride or other zinc salt giving the zinc ion is equally effective.

Water solutions of metal thiocyanates other than those of zinc and cadmium have been found helpful in enhancing the resistance of wool fibers to decomposition when heated, but the thiocyanates of zinc and cadmium are definitely superior to the others, and hence, are preferred.

## What I claim is:

- A fabric formed substantially of wool fibers and characterized by its resistance to decomposition when subjected to temperatures up to about 300° F.; said fabric having a complex, metallo-thiocyanate chemically combined with said fibers but being otherwise substantially free of other metallic compounds.
- A fabric formed substantially of wool fibers and characterized by its resistance to decomposition when subjected to temperatures up to about 300° F.; said fabric having a metal capable of

forming symmetrical complex ions with thiocyanates in water solution chemically combined with said fibers, but being otherwise substantially free of other metallic compounds.

3. The fabric set forth in claim 1 in which the metal forming said complex, metallo-thiocyanate is zinc.

4. The fabric set forth in claim 1 in which the metal forming said complex, metallo-thiocyanate is cadmium.

5. A fabric formed substantially of wool fibers and characterized by its resistance to decomposition when subjected to temperatures up to about 300° F.; in the presence of moisture; said fabric having a complex, cupric-thiocyanate chemically combined with said fibers but being otherwise substantially free of other metallic compounds.

6. The method of increasing the resistance of wool to decomposition when exposed to temperatures up to about 300° F., which consists in treating said wool in a water solution containing metal ions and thiocyanate ions until the fibers of said wool are thoroughly saturated with said solution and an organic, metallo-thiocyanate complex is formed therewith; and thereafter drying said wool.

7. The method of increasing the resistance of a textile fabric formed substantially of wool fibers to decomposition when subjected to temperatures up to about 300° F., which consists in treating said fabric in a water solution containing at least 0.07%, by weight, of a metal thiocyanate until said fibers are thoroughly saturated with said solution, and an organic, metallo-thiocyanate complex is formed therewith; and thereafter drying said fabric.

8. The method set forth in claim 7 in which the

metal forming said metal thiocyanate is a metal capable of forming a symmetrical, thiocyanate, complex ion.

9. The method set forth in claim 7 in which the metal forming said metal thiocyanate is zinc.

10. The method set forth in claim 7 in which the metal forming said metal thiocyanate is cadmium.

11. The method set forth in claim 7 in which the metal forming said metal thiocyanate is copper.

12. The method set forth in claim 7 in which the quantity of metal thiocyanate in said solution is from about 1% to about 3%, by weight.

15 13. The method set forth in claim 7 in which the temperature of said solution is maintained in the approximate range of 115° to 120° F., and the metal forming said thiocyanate is zinc.

14. The method set forth in claim 7 in which the temperature of said solution is maintained in the approximate range of 115° to 120° F., and the metal forming said thiocyanate is cadmium.

20 15. The method set forth in claim 7 in which the temperature of said solution is maintained in the approximate range of 115° to 120° F., and the metal forming said thiocyanate is copper.

CHARLES R. BARNES.

#### REFERENCES CITED

30 30 The following references are of record in the file of this patent:

#### UNITED STATES PATENTS

| Number    | Name   | Date          |
|-----------|--------|---------------|
| 1,757,519 | Ellis  | May 6, 1930   |
| 1,947,024 | Slagle | Feb. 13, 1934 |
| 2,028,769 | Ellis  | Jan. 28, 1936 |